

## UNITED STATES PATENT OFFICE

SAMUEL WEIN, OF NEW YORK, N. Y., ASSIGNOR OF ONE-HALF TO NATHAN RAFF, OF NEW YORK, N. Y.

## VISCOSE AND METHOD OF MANUFACTURING THE SAME

No Drawing.

Application filed March 1, 1924. Serial No. 696,392.

My invention relates to a new and improved method of making viscose and a new and improved viscose resulting therefrom.

One of the objects of my invention is to provide a new and improved viscose which will be slow burning and which will have considerable strength and tenacity.

Another object of my invention is to provide a new and improved method of producing a compound having the above mentioned characteristics. A preferred example of the above mentioned new and improved compound and the new and improved method of procuring the same is herewith given, it being understood that this example is merely given by way of illustration and that my invention is not limited to the details, proportions or ingredients specified therein.

I first treat 100 lbs. of cellulose, preferably ordinary cellulose derived from wood pulp, by means of the ordinary sulphite treatment. This may be the ordinary commercial wood pulp cellulose that can be secured in the open market and is preferably in the form of sheets of about the thickness of ordinary cardboard.

This is treated with an aqueous 20% zinc chloride solution at a temperature of about 5° C. I prefer to have the wood pulp at a temperature of substantially 5° C. before the said wood pulp is treated by the zinc chloride solution which is preferably kept in a tank having any well known means for maintaining the requisite temperature of about 5° C.

I first prefer to place the wood pulp in the tank and then to add enough of the zinc chloride solution to fully cover the said wood pulp in the tank.

The wood pulp is then allowed to steep in the zinc chloride solution at this temperature, for a period of about one hour and during this period I prefer not to agitate either the wood pulp or the solution. This treatment is for the purpose of converting the cellulose into a hydrated cellulose, so that the cellulose has been rendered somewhat gelatinous, so that it can be formed into blocks or sheets.

I prefer not to agitate the cellulose and zinc chloride during this period of one hour be-

cause such agitation would tend to cause the solution of the cellulose which is not desirable, as its conversion into a hydrated cellulose without solution is desired. At the expiration of this one hour period, the excess zinc chloride is drained off by any suitable means.

A sufficient quantity of 18% caustic soda solution, which has been chilled to a temperature of 5° C., is now added to the sheets of hydrated cellulose which are now in the tank. The hydrated cellulose is treated with this caustic soda solution at the above mentioned temperature of 5° C. for a period of about two hours, also preferably without any agitation.

The treatment with the caustic soda solution converts the hydrated cellulose into an alkali cellulose.

The caustic soda solution is then drained from the contents of the tank.

The sheets of treated cellulose are now subjected to high pressure in a suitable hydraulic press so that they are formed into a number of compressed blocks. The purpose of this compression is to force out all excess solution and it is believed that no chemical action is caused by means of the pressure alone. The alkali cellulose is preferably maintained at 5° C. during the compression so that the compressed blocks are also at the temperature of 5° C. The above temperature of 5° C. during the previously mentioned steps of the process is preferably secured by conducting all these operations in a room which is artificially cooled to a temperature of about 5° C.

The pressure in the hydraulic press is preferably maintained for about two hours so as to squeeze out the proper amount of excess solution.

At the end of this period the blocks are still moist and they are then disintegrated by any convenient means so as to form a mass of separated fibers which tend to cling together and have a consistency similar to that of moist bread crumbs.

The comminuted alkali cellulose is now placed in jars made of an inert substance such as porcelain and kept in these jars, which are suitably covered, for a period be-

tween seventy-two to ninety-six hours. During this period the alkali cellulose is kept at the same temperature. The longer period of aging is preferably for treating alkali cellulose having a high copper number, that is, cellulose having a high "oxycellulose" content.

The jars in which the alkali cellulose is aged are kept covered so as to prevent the absorption of carbon dioxide or other gases 10 that may be present in the atmosphere.

The aged alkali cellulose, which is a cellulose hydrate, is then placed in any suitable revolving vessel and it is there treated with carbon disulphide. I prefer to use carbon 15 disulphide in the proportion of 20 lbs. to every batch originally containing 100 lbs. of dry cellulose.

The carbon disulphide is slowly added during the period of treatment therewith and 20 the barrel containing the batch is also revolved very slowly as otherwise the carbon disulphide would tend to explode, because of the low boiling point of the carbon disulphide, and because the reaction produces 25 heat.

The treatment with the carbon disulphide is maintained for a period of about two hours and I prefer to add the carbon disulphide in 30 5 lb. batches during this period. I prefer to add the additional quantities of carbon disulphide at fifteen minute intervals and by using a sufficiently large barrel or tumbler the entire batch resulting from the original 35 100 lbs. of dry cellulose can be treated in a single barrel or tumbler with the 20 lbs. of carbon disulphide before mentioned.

The above-mentioned step of this process is carried out at the above-mentioned temperature of 5° C. as before mentioned.

40 The excess carbon disulphide is then removed as much as possible in any suitable manner from the cellulose compound formed by the action of the carbon disulphide as, for example, by allowing it to evaporate. However, since the temperature of the reaction mass must be kept quite low, namely, at a 45 temperature of about 5°, as later mentioned herein, this causes some of the carbon disulphide to remain unevaporated, so that it remains as a sulphur impurity in the solution 50 formed when the caustic soda is added, as later mentioned herein. The alkali-cellulose hydrate which has been formed previous to the reaction with the carbon disulphide, reacts with the carbon disulphide to form sodium xanthogenate which is soluble in water.

The cellulose is then placed in a tank, preferably a cast-iron tank and enough 18% caustic soda solution is added at a temperature of 60 5° C. to completely dissolve the mass of cellulose compound by forming the before mentioned sodium salt. The amount of caustic soda solution which is added at this point 65 varies according to the concentration of the

solution of the cellulose in the caustic soda which is desired.

For example, if it is desired to make an artificial silk, it is preferable to have up to 5% of the treated cellulose dissolve in the 70 18% caustic soda solution. In making a coarser thread such as, for example, imitation horsehair the concentration of the solution of the treated cellulose in the 18% caustic soda solution may be as high as 10%. 75

For making transparent sheets of material the concentration of the dissolved cellulose in the 18% caustic soda solution may be 15% and even higher.

The contaminating agents in commercially 80 manufactured products of various types include certain sulphur salts.

However, the treatment with the carbon disulphide before mentioned of an alkali cellulose hydrate made from cellulose which 85 has been previously hydrated by means of a zinc compound causes the formation of insoluble zinc salts. These last mentioned metallic salts are insoluble in the solution of the sodium salt finally formed as above mentioned, so that upon allowing the solution to stand for a suitable length of time these insoluble precipitates can be removed by any suitable filtering means or by removing the supernatant liquor. I can only state the 90 chemical reactions involved to the best of my knowledge and I do not wish to bind myself to any definite chemical theory, because the chemistry of cellulose is still obscure, but I may state my present opinion 95 of the reactions involved as follows:—

By treating the cellulose with zinc chloride, a cellulose hydrate is formed whose constitution is supposed to be  $(C_6H_{10}O_5)_x(H_2O)_y$ . When this hydrate is treated with the sodium 100 hydroxide solution, soluble sodium zincate, sodium chloride and a compound whose constitution is unknown is formed. I believe that this is a compound in which the sodium hydroxide molecule has been added to the cellulose aggregate and without resolving said aggregate. The treatment with carbon disulphide produces sodium xanthogenate, whose exact formula is unknown. The sodium zincate reacts at this point to precipitate 105 the impurities before mentioned. The subsequent treatment with sodium hydroxide solution produces the soluble sodium salt of this acid or what is known as a viscose solution, and this solution, being free from objectionable impurities, can be decomposed by various well-known solutions in the well known manner to cause reversion to what in reality is "cellulose hydrate" which may be dried and dehydrated in the well known manner. This 110 end product is a viscose of a new and improved kind.

The solution thus manufactured can now be utilized industrially by any convenient and well known methods.

The cellulose may be derived from any source in addition to the above mentioned, and my invention is not restricted to the use of zinc chloride as other solutions of metallic salts may be utilized in place of the zinc chloride and these will form insoluble metallic compounds whereby the objectionable impurities before mentioned may be either wholly or partially removed.

I believe that any hydrogen sulphide present as an impurity causes the formation and precipitation of zinc sulphide which is insoluble in the neutral or alkaline solution formed by the addition of the caustic soda solution. Likewise, if any carbon disulphide has remained as an impurity, I believe that it forms either insoluble zinc sulphocarbonate or else the carbon disulphide forms sodium sulphocarbonate, which reacts with the soluble zinc salt to form insoluble and precipitated zinc sulphocarbonate. I believe that any sodium sulphocarbonate which is present as an impurity also reacts with the soluble zinc salt to form insoluble zinc sulphocarbonate. Since the salts of other metals would produce similar reactions, I do not restrict my invention to the use of soluble zinc salt, although it is obvious that the production of a soluble zinc salt by hydrating the raw cellulose with the zinc chloride is the preferred method, because a soluble zinc chloride has a direct action in the process, and in addition the soluble zinc salt which is formed (namely, sodium zincate) is very uniformly distributed over the entire mass, so that it is not necessary to agitate the mass or the like.

I prefer to have the entire process carried out at a temperature of 5° C., by having all the implements, vessels, materials, etc. kept in a room which is artificially cooled to a temperature of 5° C. One of the important useful advantages of the new and improved cellulose solution above mentioned is that when it is desired to make a coherent sheet of cellulose hydrate therefrom, it is merely necessary to evaporate a sufficient amount of the solution in heated molds until the solvent has evaporated. As before noted, the effect of the preliminary treatment with zinc chloride is to gelatinize or "vulcanize" the cellulose. Hence, a coherent sheet of gelatinized hydrated cellulose can be formed by merely evaporating the solvent, and without the use of inorganic salts or dilute acids or the like, which have hitherto been necessary to regenerate the cellulose in the form of coherent bodies.

Similarly in forming threads from the above mentioned solution, it is necessary to squirt the said solution through fine tubes into a coagulating medium, but it is not necessary to add desulphurizing substances to this coagulating medium.

While the exact chemical nature of the

cellulose product described from the solution before mentioned, has not yet been determined, I will refer to it as "viscoid" since this is the name generally given to the regenerated cellulose which has been formed from a cellulose xanthate solution by means of inorganic salts or dilute acids. This is believed to be a cellulose hydrate.

I have described a preferred embodiment of my invention; but it is clear that the numerous changes and omissions could be made without departing from its spirit, and in particular, I claim the novel articles of manufacture or compositions specified herein, independently of the process used for making them. I cannot determine whether the viscose or viscose solution produced as before specified is entirely free from the impurities before specified and hence I will define it as being partially free therefrom.

I claim:

1. In the art of manufacturing viscose, those steps which consist in forming a soluble cellulose xanthogenate and substantially removing sulphur compounds therefrom before precipitating the viscose.

2. A method of making a viscose solution which consists in hydrating cellulose in the presence of a zinc chloride solution and without dissolving the cellulose in the zinc chloride solution, causing the hydrated cellulose containing the said zinc chloride solution to then react with an alkali solution to form an alkali-cellulose-hydrate containing a zinc salt, and causing the said alkali-cellulose-hydrate and zinc salt to react with carbon disulphide.

3. In the art of making cellulose hydrate, those steps which consist in forming a cellulose solution containing undissolved sulphur compounds therein uncombined with the cellulose, and substantially removing said compounds before reprecipitating the cellulose.

4. In the art of separating a dissolved zinc compound from gelatinized cellulose which contains said compound, those steps which consist in treating said gelatinized cellulose with a substance adapted to react with said zinc compound to form an insoluble zinc compound and removing the insoluble compound thus formed.

5. In the art of separating a dissolved zinc compound from a body of gelatinized cellulose which contains said compound, those steps which consist in causing the cellulose to react with carbon disulphide, and then forming an alkaline solution of the reaction mass in which the zinc compounds are precipitated in soluble form.

6. As a new and useful article of manufacture, a solution of an alkali metal cellulose xanthogenate resulting directly from the interaction of a soluble cellulose compound and carbon disulphide, the solution of the reaction mass having been formed in an alkaline sol-

vent without any purifying treatment for removing sulphur-containing impurities, said solution being substantially free from dissolved sulphur-containing impurities.

7. As a new and useful article of manufacture, a gelatinized viscoid free from the gelatinizing agent.

8. As a new and useful article of manufacture, a reprecipitated gelatinized viscoid.

10. In testimony whereof I hereunto affix my signature.

SAMUEL WEIN.

15

20

25

30

35

40

45

50

55

60

65